

## UNITED STATES PATENT OFFICE

ARTHUR S. ROBERTS, OF HENDERSONVILLE, NORTH CAROLINA

## METHOD OF CROSS-DYEING FABRICS

No Drawing. Application filed April 6, 1928, Serial No. 268,073. Renewed December 11, 1930.

This invention relates to new cross-dyed fabrics and to methods of preparing the same.

This application is in part a continuation 5 of my co-pending applications 240,919, 240, 920 and 240,921.

According to this invention, fabrics comprising cotton fibers and fibers of a regenerated cellulose, particularly viscose silk, are 10 cross-dyed so that the cotton and regenerated cellulose fibers are dyed different colors. It has heretofore been claimed by those skilled in the art of dyeing fabrics that a fabric composed of cotton and xanthate silk, i. e., 15 viscose silk, cannot be dyed in any other manner than that of dyeing both the cotton and the xanthate silk or viscose silk of the same color, due to the fact that cotton and viscose silk have the same affinity for dyes.

20 It is the purpose of this invention to set forth a method whereby cotton and viscose silk, or xanthate silk, can be dyed different colors when woven in the same fabric, and by dyeing each fiber in a separate dye-bath, 25 or by combining the two dye-baths and dyeing two separate and distinct colors at one and the same operation, the art of which is known as "cross-dyeing". I am aware that the art of cross-dyeing has been used here- 30 tofore for various textile articles woven of different materials, but, as stated, there has not heretofore been used any method whereby cotton and regenerated cellulose of the viscose type, when woven in the same fabric 35 can be dyed separate and distinct colors either by separate dyeing or by one operation.

The cross-dyed fabrics of the present invention are dyed in the piece and differ from 40 materials which are manufactured from fibers which have previously been dyed. The new cross-dyed fabrics comprise cotton fibers and fibers of a regenerated cellulose, and the dyeing is carried out in such a way that 45 each of these two fibers is dyed a different color. The difference in the colors produced is due to the different affinities of the dyestuffs for the different types of fiber, as will appear from what follows. Even though 50 the color of one fiber may be due to a blend

of the dyestuffs employed, the predominating color of each fiber is due to a different dyestuff.

This invention is applicable to knitted fabrics and woven fabrics comprising fibers 55 of cotton and regenerated cellulose, particularly viscose. It is applicable to fabrics in which one of these fibers is used as the warp and the other is used as the filling, and to figured fabrics in which the background may 60 be composed entirely of cotton and the figure may be composed of a regenerated cellulose, or the background may be of the regenerated cellulose and the figure of cotton. Stockings and other knitted wear comprising cotton fibers and fibers of a regenerated cellulose may be cross-dyed according to this 65 invention.

To dye the cotton fibers a dyestuff is used 70 which has a preferential affinity for cotton in the presence of the regenerated cellulose employed, and this dyestuff is applied to the fabric in such a way that in the final product this dyestuff gives the predominating color 75 to the cotton, although the color of the cotton may in fact be due to a blend of this dyestuff with the dyestuff used to give the predominating color to the regenerated cellulose. Similarly, to dye the regenerated cellulose fibers a dyestuff is used which has a 80 preferential affinity for the regenerated cellulose, and although the color of the regenerated cellulose fibers may be due to a blend of dyestuffs, the predominating color 85 of these fibers is produced by this dyestuff.

Not all dyestuffs give an even dyeing 90 when applied to fabrics comprising cotton fibers and fibers of regenerated cellulose, e. g., viscose silk. Certain dyestuffs exhibit a decided preferential affinity for one or the other type of fiber during the dyeing treatment. In dyeing with certain dyestuffs this preferential affinity may be emphasized by employing a higher or lower temperature 95 during the dyeing treatment. For example, in cross-dyeing a fabric composed of cotton and regenerated silk fibers, it is desirable to employ a high temperature when dyeing with certain dyestuffs having a preferential affinity for viscose silk, and a lower tempera- 100

ture in dyeing with certain dyestuffs having a preferential affinity for the cotton, as will more fully appear from the examples given below.

- 5 In cross-dyeing according to this invention, it is not necessary that the dyestuffs employed should dye one of the fibers a deeper shade than the other during the dyeing operation. A dyestuff may be used 10 which distributes itself more or less evenly over both types of fiber in the dye-bath, if the dyestuff is more closely held by one of the fibers than the other so that when subjected to a clearing treatment, such as boiling 15 with soap, or washing in a hot soap bath, the dyestuff will be sufficiently removed from one fiber to allow the production of cross-dyed effects by subsequently dyeing with a dyestuff of different color showing a 20 preferential affinity for the fiber retaining the least amount of the first dyestuff. For example, a dyestuff may give a fairly even dyeing on a fabric comprising cotton and viscose silk fibers. If, on subsequently boiling 25 the fabric with soap, or otherwise clearing, this dyestuff is almost entirely removed from one of the fibers, e. g., the cotton, so that a cross-dyed fabric may be obtained by dyeing the soaped fabric with a dyestuff having 30 such a preferential affinity for the cotton that on dyeing it dyes the cotton a deeper shade than the viscose silk, such a dyestuff may be used in cross-dyeing because it has a preferential affinity for viscose silk.
- 35 When a separate dye-bath is used for each of the dyestuffs employed in cross-dyeing according to this invention, even though a decided two-tone effect is produced on the fabric during the first dyeing operation, without subsequent treatment, it is often desirable to subject the fabric to a clearing operation between the two dyeing operations in order to at least partially remove the color from the fiber which it is intended 40 should be dyed to the least extent in the first dye-bath. In general, a hot soap bath will satisfactorily clear the color from cotton and not detrimentally affect the color on the viscose silk. Turkey red oil may be 45 added to the soap-bath. Hydrochloric acid may be used to clear certain basic colors from cotton. The examples given below illustrate applications of such a clearing step.
- 50 According to the present invention, the different affinities exhibited by the different dyestuffs are utilized to advantage in order to produce materials in which the different fibers are dyed different colors. It has been 55 found that by carefully selecting two dyestuffs, attractive cross-dye pieces may be prepared in which cotton is dyed one color and viscose silk another. Dyestuffs of various 60 classes have been found to give satisfactory 65 results.

*Example I.*—I have found that certain substantive dyestuffs, for example, direct rubine B concentrated Schultz Number 313, will when combined with certain vegetable oils such as castor oil, pine oil, balsam oil, turpentine and the like to the approximate amount of about 66 $\frac{2}{3}$ % of the oils, singly or in combination and 33 $\frac{1}{3}$ % of the dyestuff will form a paste that when entered into the dye machine containing sufficient water at 70 a temperature of approximately 120° F., together with the usual amount of sodium chloride and soap forms a dye-bath which will dye the cotton to the color and shade desired and leave the xanthate silk or viscose 75 only slightly tinted. I have also discovered that by using wool blue R Schultz Number 188 when combined with glycerine in the approximate proportion of 66 $\frac{2}{3}$ % of the glycerine and 33 $\frac{1}{3}$ % of the dyestuff will form 80 a paste that when introduced into a dye machine containing sufficient water at a temperature of approximately 130° F., together with the usual amount of sodium sulfate and "boil-off oil" as is used in some cases, will 85 form a dye-bath that will dye a viscose or xanthate silk to the color and shade desired and leave the cotton only slightly tinted. If a fabric comprising viscose silk and cotton fibers is entered into the dye-bath containing 90 the direct rubine B concentrated and the vegetable oils, which dyes cotton, the fabric can, after having been washed to remove the surplus dye, be introduced at once into the dye-bath containing the acid dyestuff, that 95 is, the wool blue R and the glycerine and the viscose or xanthate silk will be dyed a distinct color, thus producing the two-color or cross-dye effect which heretofore has never 100 been accomplished with these materials.

A fabric comprising viscose silk and cotton may likewise be dyed with a direct dyestuff and an acid dyestuff without the use of vegetable oils or glycerine. For example, a fabric comprising cotton and viscose silk 105 fibers after being properly washed to remove oils and after wetting may be entered into a bath of direct rubine B concentrated Schultz Number 313, and the bath held at a temperature of approximately 120° F., or lower, until the cotton is dyed. The fabric is then rinsed and entered into a bath of the proper concentration of wool blue R Schultz Number 188 and held at a temperature of 110 approximately 130° F., until the viscose is 115 dyed to the proper shade.

*Example II.*—It is known that two shades of the same color can be produced on cotton-viscose silk fabrics with basic dyestuffs. Rhodamine 6G extra Schultz Number 571, 120 rhodamine B Schultz Number 573 and Schultz Number 571 rhodamine 6G have been used for this purpose. Nevertheless, it is new, so far as I am aware, to cross-dye 125 cotton-viscose silk material using a basic 130

dyestuff to give the predominating color on the viscose silk and then applying a direct color with a preferential affinity for cotton to produce the cross-dye effect. Rhodamine 6G extra Schultz Number 571 may be used to dye the viscose silk. From three to five percent acetic acid, formic acid, or sulfuric acid (32° Tw.) may be placed in the dye-bath and the necessary water added. The dissolved basic dyestuff is then poured into the dye-bath which is heated to approximately 180° F. The goods are then run into the machine and given from three to five "ends" or dips in the dye liquor, or any number required to produce a shade of sufficient depth. The dye-bath is then run off and then the goods given a thorough washing in cold water.

The direct dyestuff is dissolved and added to sufficient water in the machine heated to approximately 120° F., direct yellow S2G Schultz Number 351 or direct rubine B concentrated Schultz Number 313 may be used. The dyestuff is entered and the goods are run in and given e. g. three to five "ends" or dips for the purpose of bringing up the shade desired on the cotton fibers in the fabric. This dye-bath is then run off and the goods are given a thorough rinsing to clear the fabric of the surplus dyestuff and then squeezed and dried.

In addition to the rhodamines the following basic dyestuffs may be used; methyl violet Schultz Number 515, Victoria blue 35 Schultz Number 559, methylene blue Schultz Number 659, Astra phloxine F. F. extra Schultz Number 596, brilliant green crystals Schultz Number 499 and malachite green, Schultz Number 495.

Other direct dyestuffs having a preferential affinity for cotton in the presence of viscose silk, may be used. Such dyestuffs include direct rubine B concentrated Schultz No. 313, direct yellow S2G Schultz No. 10, direct fast blue 6GL Schultz No. 456, diazo sky blue B Schultz No. 337, Pontamine diazo blue 3G Schultz No. 471, diazo blue BR Schultz No. 274, diazo blue O Schultz No. 326, diazo blue 2RL Schultz No. 274, diazo blue NA Schultz No. 273, cotton fast yellow A, Schultz No. 9, azo navy blue Ex Schultz No. 337, cotton fast orange 5R Schultz No. 11, aminil fast yellow A Schultz No. 9, Jenyl orange Schultz No. 11 and chloramine green B Schultz No. 470.

The direct dyestuff is preferably applied at a temperature in the neighborhood of 120° F. It may be preferable to have a small amount of sodium hydroxide in the bath containing the direct dyestuff. Although here described as applied to jigg dyeing the process may at times be more advantageously carried out in dye-becks.

After dyeing with the basic dyestuff and before applying the direct dyestuff, it may

be advisable to treat the two-tone fabric in such a way as to clear the color from the cotton. The desirability of such a treatment is greater in certain instances than in others. Certain basic dyestuffs exhibit such a preferential affinity for viscose, especially when dyeing light shades, that little color goes to the cotton, and in such a case it may not be necessary to clear the fabric between applications of the dyestuffs. Where desirable, hot soap or dilute hydrochloric acid may be used to clear the color from the cotton.

*Example III.*—Two direct dyes each of which exhibits the proper preferential affinity for a different fiber may be used to cross-dye a fabric comprising cotton and viscose silk fibers. After properly conditioning the material it is immersed in a dye-bath containing the dyestuff with a preferential affinity for the viscose silk, e. g., naphthamine brilliant blue G extra Schultz Number 877, while the dye-bath is held at a temperature of about 190° F., to boiling. The dye stains the cotton but dyes the viscose silk a much deeper shade than the cotton. This viscose silk is dyed to the desired shade. The fabric is then preferably rinsed with cold water before applying the dyestuff with a preferential affinity for the cotton. Before dyeing the cotton, it may be desirable to boil the goods with soap or otherwise treat them to clear the color from the cotton, and then rinse. The fabric is then immersed in the dye-bath containing a direct dyestuff such as direct rubine B Schultz Number 313 concentrated, which has a preferential affinity for cotton in the presence of viscose silk. Other direct dyestuffs mentioned in connection with Example II may be used. The bath is kept at a temperature of about 90 to 110 or 120° F. An addition of a small amount of sodium hydroxide to this latter bath gives good results. When sodium hydroxide is used, a final rinse in an acid bath may be used to remove any caustic. In the absence of sodium hydroxide, the cloth, after dyeing in the second dye-bath, is merely rinsed in cold water and dried. Glauber's salt, sodium phosphate or sodium chloride may be added to either or both of the baths to get better exhaustion of the color from the bath on to the fabric; but the addition of such salts is not necessary and it appears to have no appreciable effect on the cross-dyeing.

Instead of naphthamine brilliant blue G Ex Schultz No. 323, diphenyl red FC Schultz No. 343, primuline Schultz No. 616, may be used. Other direct dyestuffs which have a preferential affinity for viscose silk in the presence of cotton and may be used are: Jenyl red SGM Schultz No. 194, diamine fast scarlet B, Schultz No. 319, triazol

brilliant sky blue 6B, Schultz No. 426, cotton grey B, Schultz No. 241, amidine fast black FF, Schultz No. 436, and Jenyl fast black GG, Schultz No. 462.

- 5 Attractive fabrics may be prepared by dyeing the viscose silk with naphthamine brilliant blue G extra and dyeing the cotton with direct rubine B concentrated, direct yellow S2G, C R cotton fast yellow A or C R 10 cotton fast orange 5R, according to the combination of colors desired. The shade to which each fiber is dyed may be regulated in the usual manner by controlling the concentration of the dye-bath or the length of 15 the dyeing operation, etc.

If a pink or red is desired on the viscose, diphenyl red S C may be used, and any one of the following may be used on the cotton to produce the combination of colors desired: 20 Direct yellow S2G, cotton fast yellow A, cotton fast orange 5R, direct fast blue 6GL, and cotton fast blue 4GL.

Primuline may be used to dye the viscose a desired shade of yellow and then direct 25 rubine B concentrated, direct fast blue 6GL or cotton fast blue 4GL may be used to produce the desired color on the cotton. Other pleasing color combinations may be obtained by selecting other combinations 30 from the dyestuffs listed above.

*Example IV.*—A fabric comprising fibers of cotton and viscose silk may be cross-dyed using direct dyes with a preferential affinity for the cotton in the presence of viscose silk 35 and developed colors which have a preferential affinity for viscose silk in the presence of cotton. Both dyestuffs may be applied from the same dye-bath, or two separate dye-baths may be used, in which case a clearing 40 step may be included between the two dyeing treatments.

To illustrate—Primuline and direct rubine B concentrated may be dissolved and added to the same dye-bath. As a specific 45 example, in the dyeing of 100 pounds of material, four ounces of primuline and 12 ounces of direct rubine B concentrated may be dissolved and added to 40 gallons of water. The dye-bath is brought to a temperature 50 of approximately 140° F., and the goods are given from three to five "ends" or dips when jiggs are used, or a corresponding treatment may be given in a dye beck. The goods are then rinsed and the primuline is diazotized 55 with an acid solution of nitrite. A solution of 1.5-2.5% sodium nitrite and 5-7.5% hydrochloric acid or 3-5% sulfuric acid may be used. The primuline is then developed. A developer may be used which will give a 60 desired color on viscose silk to harmonize with the color produced on the cotton. A sodium hydroxide solution of phenol used as a developer will give a yellow color. Resorcin will give orange. Naphthylamine 65 ether N powder will give blue. If, instead

of direct rubine B concentrated, direct yellow S2G is used, the cotton will be dyed yellow and red may be produced on the viscose silk by developing with betanaphthol.

Thus, by combining the two dye-baths, 70 diazotizing and developing, two separate and distinct colors may be dyed on a fabric composed of viscose silk and cotton from the same dye-bath.

Instead of applying both colors from the same dye-bath, it will generally be preferable to employ separate dye-baths. The viscose silk may be dyed first, and then the cotton. For example, a fabric composed of cotton and viscose silk threads may be wet 75 out in cold water in the usual way and left in a roll on the dye machine. The machine is filled with water which is heated to approximately 160° F., or higher, and the developed dyestuff, after having been dissolved in a small amount of water, is poured into the machine. The dyestuff is preferably 80 added in two parts, one-half after the first "end" or dip, and the remaining one-half after the second "end" or dip, after which 85 the goods are given as many "ends" as is desired to bring up the shade. As a developed dyestuff having a preferential affinity for viscose in the presence of cotton, 90 primuline may be selected as an example. 95

After subjecting the cloth to the dye-bath for the desired length of time, the bath is run off and the goods are rinsed, preferably in cold water, and the primuline or other developed dyestuff is diazotized, as explained 100 above in connection with the application of a developed dyestuff, together with a direct dyestuff from the same bath. The dyestuff is diazotized and coupled in the usual manner. The developing bath comprising the developer is applied to the fabric after the diazotization and the developer used may be selected with a view to producing a color 105 on the viscose silk which will properly harmonize with the color to be later produced on the cotton. The goods are then washed with water and it is preferable to soap the goods in a warm bath and clear as much of the developed color as possible from the cotton before applying the direct dyestuff having a preferential affinity for the cotton. The goods are then rinsed in cold water, or 110 may preferably be first treated in a bath which is slightly acid in order to remove any trace of alkalinity from the goods. 115

The dye-bath for coloring the cotton portion of the fabric is then made up by dissolving a direct dyestuff in sufficient water, and the goods are given a sufficient number of dips or "ends" at a temperature in the 120 neighborhood of 120° F., to produce the color and shade desired on this part of the fabric. The direct dye stuff used may be direct yellow S2G or another of the direct dyestuffs suggested in connection with Ex- 125 130

ample II, in which a basic dyestuff and a direct dyestuff are applied to a cotton-viscose silk fabric. After applying the direct dyestuff, the goods are given a thorough washing, preferably in cold water, and then 5 squeezed and dried.

*Example V.*—Primuline exhibits a preferential affinity for viscose silk fibers in the presence of cotton fibers. Other developed 10 colors exhibit a preferential affinity for cotton in the presence of viscose silk. Two properly selected developed colors may be used for producing cross-dyed effects on viscose silk. Primuline, for example, may be 15 applied to the viscose silk. After applying the primuline at a temperature near the boiling point of the dye-bath, and preferably after boiling down with soap or otherwise clearing, the color may be developed and 20 then the developed color with a preferential affinity for cotton, e. g., diazo sky blue B may be produced on the cotton, using a warm bath with a temperature in the neighborhood of 90-115° F., or higher. Any one 25 of the following colors may be used to dye the cotton; diazo sky blue B, direct diazo blue 3G, direct diazo blue B R, direct diazo blue RRL, direct diazo blue O, direct diazo blue NA, and diazo blue 2RL. These colors 30 are developed by coupling with the developers known in the art. For instance, when a blue is desired, diazo sky blue B may be developed with betanaphthol.

Although generally better results will be 35 obtained by using a separate dye-bath for each color, it is possible to apply both dyestuffs in one bath. After diazotizing, the dyestuffs will be developed with the same developer. For example, primuline may be 40 used for giving the predominating color to the viscose silk, and diazo sky blue B for the cotton. These will be applied to the fabric from the same bath at a temperature of approximately 160° F. After rinsing, the fabric 45 is immersed in a diazotizing bath and then beta naphthol may be used to develop red on the viscose silk and blue on the cotton. When the two-bath method is utilized, i. e., when one color is developed before the 50 other is applied, different developers may be employed. It is possible to first treat the cloth with a developed color with a preferential affinity for the viscose silk, such as primuline, clear, and then apply a developed 55 color with preferential affinity for the cotton, and then diazotize and develop both with the same developer.

Those developed colors exhibiting a preferential affinity for cotton, listed above in 60 connection with Example V, may be used together with dyestuffs of various classes for coloring viscose silk to produce attractive cross-dyed pieces, as more fully brought out in Examples VI and VII.

*Example VI.*—A cotton-viscose silk fab-

ric may be treated with naphthamine brilliant blue G extra to color the viscose silk in the manner described in Example III. One of the other direct dyestuffs listed in that example for dyeing viscose silk in the 70 presence of cotton may be used. After clearing the dyestuff from the cotton by boiling with soap or other suitable clearing agent, the cotton is dyed with a developed dyestuff having a preferential affinity for the cotton, 75 e. g., diazo sky blue B, at a temperature of about 95-110° F., and diazotized and coupled with a desired developer.

*Example VII.*—A basic dyestuff having 80 a preferential affinity for viscose silk in the presence of cotton, may be used for dyeing the viscose silk at a temperature near the boiling point of the dye-bath, and then preferably after clearing, a developed color may be applied to the cotton in the manner described above in connection with Example V. As a specific example, rhodamine 6G extra may be applied to the viscose in the manner described in Example II and then pon- 85 tamine diazo blue 3G may be used to give 90 the predominating color to the cotton. The blue may be developed with beta naphthol. Although the developed color is preferably dyed from a temperature bath it may be dyed 95 hot.

The foregoing examples are set forth in such a way as to supply one skilled in the art with the information necessary to cross-dye textile materials composed of fibers of cotton and a regenerated cellulose. 100

It will thus be seen that various classes of dyestuffs may be used for producing the desired color on either of the fibers and various processes may be used. Several dyestuffs may be used to produce a desired color 105 on one fiber. The viscose silk may be dyed first, then the cotton, or the reverse order may be followed, or dyestuffs showing a preferential affinity for cotton and viscose silk in the presence of each other may be applied from the same bath. The dyestuffs may be used alone in the bath or where desirable the dyestuffs may be used together with oils, etc., as described in connection with the process of Example I. Ex- 110 hausting agents, such as Glauber's salt, common salt, etc., may be used and bluestone may be used in the usual manner to give a desired overtone. Acetyl cellulose, silk, wool or other fibers, may be employed together with the regenerated cellulose and cotton, and the whole may be cross-dyed to 115 give three or more colors.

Other devices known to the person skilled 120 in the art may be employed in producing the cross-dyed textile materials covered by this invention.

The dyestuffs and processes listed above 125 are illustrative of this invention and the invention is not to be considered as limited 130

thereto, but is to be construed as defined in the following claims.

I claim:

1. The process of cross-dyeing a cotton-regenerated cellulose textile fabric which comprises subjecting the fabric at a temperature near the boiling point of the dye-bath to a dyeing treatment with a dyestuff selected from the group consisting of Schultz Numbers 323-194-343-616-319-426-241-436 and 462, having a preferential affinity for the regenerated cellulose in the presence of the cotton and thereafter subjecting the fabric at a lower temperature to a dyeing treatment with a dyestuff selected from the group consisting of Schultz Numbers 313-10-326-273-471-274-9-337-11-456-470, having a preferential affinity for the cotton in the presence of the regenerated cellulose.
2. The process of cross-dyeing a cotton-regenerated cellulose textile fabric which comprises subjecting the material at a temperature near the boiling point of the dye-bath to a dyeing treatment with a dyestuff selected from the group consisting of Schultz Numbers 323-343-194-616-319-426-241-436 and 462, having a preferential affinity for the regenerated cellulose in the presence of the cotton, washing with a hot soap solution, and thereafter subjecting the fabric at a lower temperature to a dyeing treatment with a dyestuff selected from the group consisting of Schultz Numbers 313-10-326-273-471-274-9-11-456-337 and 470 having a preferential affinity for the cotton in the presence of the regenerated cellulose.
3. The method of cross-dyeing a textile fabric comprising fibers of cotton and a regenerated cellulose of the viscose type, which comprises subjecting the fabric to the action of a direct dyestuff selected from the group consisting of Schultz Numbers 323-194-343-616-319-426-241-436 and 462, with a preferential affinity for one of these two fibers in the presence of the other and subjecting the fabric to the action of a dyestuff selected from the group consisting of Schultz Numbers 313-10-326-273-471-274-9-11-456-337 and 470 having a preferential affinity for the other of the two fibers in the presence of the other fiber.
4. The method of cross-dyeing a textile fabric comprising fibers of cotton and a regenerated cellulose which comprises subjecting the fabric at a temperature in the neighborhood of 90 to 120° F., to the action of a direct dyestuff selected from the group consisting of Schultz Numbers 313-10-326-273-471-274-9-11-456-337 and 470 and also subjecting the material to the action of a dyestuff selected from the group consisting of Schultz Numbers 323-343-194-616-319-426-241-436 and 462 with

a preferential affinity for the regenerated cellulose in the presence of the cotton.

5. The method of cross-dyeing a textile fabric comprising both cotton and viscose silk which comprises subjecting the fabric to the action of a direct dyestuff selected from the group consisting of Schultz Numbers 323-343-194-616-319-426-241-436 and 462 with a preferential affinity for viscose silk in the presence of cotton at a temperature near the boiling point of the dye-bath and subjecting the fabric to the action of a direct dyestuff selected from the group consisting of Schultz Numbers 313-10-326-273-471-274-9-11-456-337 and 470 with a preferential affinity for cotton in the presence of viscose silk at a lower temperature.

6. The method of cross-dyeing a textile fabric comprising both cotton and viscose silk which comprises subjecting the fabric to the action of a direct dyestuff selected from the group consisting of Schultz Numbers 323-343-194-616-319-426-241-436 and 462 with a preferential affinity for viscose silk in the presence of the cotton at a temperature near the boiling point of the dye-bath, washing with a hot soap solution to partially clear the color from the cotton and thereafter subjecting the fabric to the action of a direct dyestuff selected from the group consisting of Schultz Numbers 313-10-326-273-471-274-9-11-456-337 and 470 with a preferential affinity for the cotton in the presence of viscose silk at a lower temperature.

In testimony whereof I affix my signature.

ARTHUR S. ROBERTS.

105

110

115

120

125

130